

Oct. 24, 1950

J. A. H. HART

2,527,263

PHOTOGRAPHIC TRANSFER MATERIALS BEARING GELATIN ANION  
SOAP COMPLEX SILVER HALIDE LAYER

Filed Nov. 15, 1946



*Fig. 1*



*Fig. 2*

INVENTOR.  
JOHN ALFRED HENRY HART  
BY

*Lynn Barrett Morris*  
ATTORNEY

## UNITED STATES PATENT OFFICE

2,527,263

PHOTOGRAPHIC TRANSFER MATERIALS  
BEARING GELATIN ANION SOAP COM-  
PLEX SILVER HALIDE LAYERJohn Alfred Henry Hart, Ilford, England, assignor  
to Ilford Limited, Ilford, England, a British  
companyApplication November 15, 1946, Serial No. 710,231  
In Great Britain November 19, 1945

4 Claims. (Cl. 95—8)

1

This invention relates to photographic materials and particularly to transfer materials from which a photographic light-sensitive emulsion layer may be transferred to another support.

Processes have been described for the production of templates and other manufactured articles wherein a photograph is formed on a support which is subsequently to be cut to the shape dictated by the photographic image. The supports are usually of metal, wood or a synthetic plastic.

Photographic materials in which the emulsion layer is carried on a temporary support and from which the emulsion layer may be transferred to a permanent support are well known. It is possible to form the latent image in the emulsion, process it while still on the temporary support and then transfer the processed image to the permanent support, but in many instances, especially where dimensional accuracy is important, it is preferable to transfer the emulsion layer to the permanent support before it is processed and to carry out the processing while it is on the permanent support since the dimensions of the permanent support are usually stable.

Unfortunately, ordinary gelatin photographic emulsions do not adhere very well to metal supports. It has therefore been proposed to provide the permanent metal support, and also the emulsion layer, with an over-coating of a lacquer, usually a nitrocellulose lacquer, and then to secure adhesion by softening the lacquer layers, pressing them together, allowing the assembly to dry, and then stripping off the temporary support (which is usually paper). Another method is to soften the lacquer coatings by heating.

This method requires that the manufacturer of the transfer material provides an outer coating of lacquer on the emulsion.

The present invention is concerned with an improved transfer material which avoids the necessity for a lacquer coat over the emulsion.

According to this invention a transfer material comprises, in order, a temporary support, preferably of paper, an adhesive "dry-stripping" layer; and a layer of a photographic emulsion comprising a dispersion in an organic solvent medium of a complex formed between gelatin and an anion soap or a sulphonate acid having a highly hydrophobic radicle in the anion, said dispersion including dispersed light-sensitive silver halide.

By the expression "dry-stripping" layer is meant a layer which may be broken down by

2

pulling apart the layers on either side of it, by manual force at ordinary temperatures and without the application of any liquid.

The production of photographic emulsions of the type just defined is described in U. S. application No. 623,445, filed October 19, 1945, to which reference may be made for the full details. Briefly the method consists in forming an emulsion of silver halide in an aqueous solution of gelatin, adding to such emulsion an anion soap or a sulphonate acid having a highly hydrophobic radicle in the anion in sufficient quantity to cause precipitation of a complex of the gelatin and the added substance, the said complex containing the dispersed silver halide, and then redispersing the complex in a predominantly organic solvent medium. Preferably the anion soap or sulphonate acid is added to the gelatin at a pH below the isoelectric point of the gelatin or in the presence of an electrolyte. There may be included in a photographic emulsion so formed a proportion of another colloid which is soluble in the organic solvent medium or which is soluble in a solvent medium which is miscible with the solvent medium already present to form a stable dispersion. Such other colloids may be, for example, cellulose esters, e. g., cellulose nitrate, cellulose acetate, far-hydrolysed cellulose esters (e. g., cellulose acetate having an acetyl content of 20-30%), polyvinyl acetate, polyvinyl acetals, methyl methacrylate polymers and the partial hydrolysis products thereof, and mixed interpolymers such as the interpolymers of maleic acid or anhydride with styrene or methyl methacrylate.

Suitable anion soaps and sulphonate acids containing highly hydrophobic radicles in the anions are listed in application No. 623,445. They include:

(a) Soluble salts of long-chain-alkyl sulphonic acids.

(b) Soluble salts of sulphated higher fatty alcohols, e. g., soluble salts of fatty alcohol sulphates of which the alkyl group contains at least 8 carbon atoms, as for example the soluble salts of lauryl hydrogen sulphate and oleyl hydrogen sulphate.

(c) Soluble salts of sulphated secondary alcohols containing at least 8 carbon atoms in the chain.

(d) Soluble salts of alkylated aromatic sulphonate acids, e. g., soluble salts of alkyl benzene sulphonate acids, of alkyl naphthalene sulphonate acids and of alkylated hydroxy diphenyl sulphonate acids.

(e) Soluble salts of long-chain-alkyl esters of sulphated succinic acid.

Thus, it will be seen that anion soaps containing sulphonic or sulphuric acid groups are preferred to those containing carboxylic acid groups.

The soluble salts may be formed from alkali metals, e. g., sodium and potassium, from ammonia or from amines, e. g., triethanolamine and cyclohexylamine.

The anion soaps may contain amino residues in the anion of the soap as, for example, in the sodium salt of oleyl amino ethane sulphonic acid which contains a carbonamide ( $-\text{NH.CO}-$ ) group.

The expression "long-chain-alkyl" is intended to mean at least 8, and preferably at least 12, carbon atoms in the alkyl group.

Very many anion soaps are commercially marketed as detergents and these commercial products may conveniently be employed in the process of this invention. Thus, suitable commercial products are the compounds sold under the trade names:

|                            |                                                               |
|----------------------------|---------------------------------------------------------------|
| Agral N -----              | The sodium salt of alkyl naphthalene sulphonic acid.          |
| Aresklene 375 -----        | The sodium salt of alkyloxy-diphenyl disulphonic acid.        |
| Dispersol L -----          | The sodium salt of dinaphthyl-methane disulphonic acid.       |
| Gardinol -----             | Sodium alkyl sulphate.                                        |
| Igepon T -----             | The sodium salt of oleoyl-methyl-amino-ethane sulphonic acid. |
| Lissapol A -----           | Sodium hexadecyl sulphate.                                    |
| Lissapol C -----           | Sodium hexadecyl sulphate.                                    |
| Lissatan A -----           | Sodium hexadecyl sulphate and formaldehyde.                   |
| Lohrinol -----             | Sulphonated fatty acid.                                       |
| Nekal A -----              | The sodium salt of alkyl naphthalene sulphonic acid.          |
| Nekal BX -----             | The sodium salt of alkyl naphthalene sulphonic acid.          |
| Perminal W -----           | The sodium salt of alkyl benzene sulphonic acid.              |
| Santomerse D -----         | The sodium salt of alkyl benzene sulphonic acid.              |
| Sulphonated Lorol TA ----- | Triethanolamine dodecyl sulphate.                             |
| Sulphonated Lorol NH ----- | Ammonium dodecyl sulphate.                                    |
| Sulphonated Lorol CY ----- | Cyclohexylamine dodecyl sulphate.                             |
| Teepol X -----             | Sodium alkyl sulphates.                                       |
| Tergitol 4 -----           | Sodium secondary alkyl sulphate.                              |
| Tergitol 7 -----           | Sodium secondary alkyl sulphate.                              |

There may be used, instead of the anion soap itself, the free acid derived from such soap.

As indicated above, instead of true anion soaps, sulphonic acids of which the anion is highly hydrophobic may be employed. These may be simple acids, for example 2-naphthol-1-sulphonic acid, 1-naphthol-4-sulphonic acid or anthraquinone-2-sulphonic acid, or may be more complex, for example dyestuffs such as Kiton Fast Yellow 3G (Colour Index No. 645) which contains a sulphophenyl-pyrazolone radicle, and Naphthalene Orange GS (Imperial Chemical Industries Ltd.) By Colour Index is meant "Society of Dyers and Colourists Colour Index," edited by F. M. Rowe, D. Sc., F. I. C., first edition, January, 1924, published by The Society at the General Offices, 30

Pearl Assurance Buildings, Bradford, Yorkshire.

In general it is preferred to form the complex from an aqueous gelatino-silver halide emulsion which has already been washed and digested.

Generally speaking the most suitable organic solvents for dispersing the complexes are those containing hydroxy groups, e. g. methyl and ethyl alcohols, ethylene glycol mono methyl ether, ethyl lactate and diacetone alcohol. Organic solvents not containing hydroxy groups are generally only useful together with some water or some hydroxy solvent, e. g. acetone, methyl ethyl ketone, dioxane, methylene chloride, chloroform and mesityl oxide are preferably used in admixture with water or methyl alcohol. Small quantities of esters, e. g. methyl acetate, butyl acetate, ethers, e. g. diethyl ether, and hydrocarbons, e. g. benzene and toluene, may also be included in the solvent medium. The choice of solvent will depend on the particular nature of the complex. Complexes formed at low pH and containing a relatively low proportion of the anion soap (or corresponding acid) are generally more easily soluble in polar solvents or in solvents containing some water, whilst those formed at higher pH values and containing more anion soap (or corresponding acid) are generally soluble in non-polar solvents, e. g. toluene. The complexes may be swollen in the organic solvent medium and dispersion is usually facilitated by gentle warming.

Any of the specific emulsions described in the aforesaid application No. 623,445 may be employed in the present invention.

The photographic emulsion layers of the transfer materials of the present invention may be transferred to metal (e. g. steel, aluminium, brass, copper or nickel), wood, plastic or other surfaces as required. Generally it is desirable that the surface to which the emulsion is to be transferred should have a lacquer surface, e. g. cellulose nitrate, cellulose acetate, polymethyl methacrylate or polyvinyl acetate. Where the surface to which the emulsion is to be transferred consists of such a plastic, softening of the actual surface of the material by the application of a solvent or by heat is usually sufficient to secure adhesion, no separate application of a lacquer layer being necessary.

The following examples illustrate the production and use of transfer material according to this invention:

#### Example 1

55 1000 gms. of a silver iodobromide emulsion containing 100 gms. gelatin was immersed in 650 cc. of water and melted down. To this was added 125 cc. of normal hydrochloric acid and 175 cc. of Teepol X (a commercial anion soap comprising a mixture of sodium alkyl sulphates). A complex of the gelatin and the anion soap, holding the silver iodobromide in suspension, was precipitated, and this was washed with 2 litres of water, drained, dissolved in 500 cc. of warm ethyl alcohol (64° O. P.) and then re-precipitated by adding 375 cc. of distilled water. The precipitate was then drained and dissolved in 1½ litres of warm ethyl alcohol (64° O. P.).

A paper base was coated with a 5% solution of beeswax in trichlorethylene and dried. It was then coated with the emulsion prepared as above and again dried. The resulting photographic transfer material is shown in section in Fig. 1 of the drawing wherein paper 1 has beeswax layer 2 coated on one surface which carries the

light-sensitive layer 3 of silver halides dispersed in the gelatin anion soap complex.

A sheet of metal was lacquered with a cellulose nitrate lacquer and allowed to dry. The lacquer layer was softened by the application of a solvent mixture consisting of equal volumes of methyl alcohol and ethylene glycol monomethyl ether applied with a swansdown pad. The transfer material was then applied to the metal sheet with the emulsion side in contact with the softened lacquer surface, the assembly pressed and allowed to dry out for one hour. The paper base was then stripped away, leaving the emulsion adhering firmly to the metal sheet.

*Example 2*

400 gms. of a silver iodobromide emulsion containing 40 gms. gelatin was melted at 110° F. and mixed with 20 gms. of diatomaceous earth ground in 200 cc. of 2% gelatin solution. To this was added 50 cc. of normal hydrochloric acid and 70 cc. of Teepol X. The resulting precipitate was separated, washed with water, drained and added to 200 cc. methyl alcohol. The temperature was raised to 125° F. and the mixture stirred until the precipitate had all dissolved. To the product was added 150 cc. distilled water and the resulting precipitate thoroughly drained. The precipitate was then dissolved in 300 cc. of ethylene glycol monomethyl ether and to this was added 30 gms. of collodion cotton HM 15/20, manufactured by Imperial Chemical Industries Limited, made into a slurry with 300 cc. butyl alcohol and 60 cc. of diacetin. The mixture was stirred for 40 minutes at 125° F. and then allowed to cool. It set to a jelly.

This stock jelly was used to make up an emulsion for coating by melting 250 gms. of the jelly at 125° F. and adding it to 750 cc. of methyl alcohol at 110–115° F. This was allowed to cool, making about 1 litre of emulsion suitable for coating.

This emulsion was coated on a beeswaxed paper support as in Example 1 and yielded a transfer material of similar value for transferring an emulsion to a lacquered metal support. The resulting transfer material is shown in Fig. 2 of the drawing adjacent to a metal sheet 4 bearing lacquer layer 5. The sheet and transfer material are shown in section and the former consists of paper support 1 bearing beeswax layer 2 which carries light-sensitive layer 3' composed of silver halides dispersed in a mixture of the complex of gelatin and the anion soap with collodion cotton.

*Example 3*

A zinc sheet was coated with the thermoplastic lacquer:

|                              |     |     |
|------------------------------|-----|-----|
| Polyvinyl acetate (Gelvo 1½) | gm. | 40  |
| Tri-cresyl phosphate         | cc. | 5   |
| Ethyl acetate                | cc. | 100 |
| Butyl acetate                | cc. | 50  |

When dry and non-tacky, the emulsion coated paper of Example 2 was pressed into contact with it (emulsion side to lacquer surface) by an iron heated to above 110° C. for about 10 seconds. Immediately the iron was removed, the assembly was rolled with a rubber roller to squeeze out air bubbles and, after cooling, the paper support was stripped away, leaving the emulsion attached to the metal sheet. Adhesion was good during processing and when dried.

*Example 4*

A brass sheet was coated with the lacquer:

|                                                                   |     |      |
|-------------------------------------------------------------------|-----|------|
| Polyvinyl acetate (Gelva 25)                                      | gm. | 15   |
| Collodion cotton HX 30/50 (damped with 30% W/W methylated spirit) | gm. | 5    |
| Triacetin                                                         | cc. | 12   |
| Acetone                                                           | cc. | 170  |
| Butyl acetate                                                     | cc. | 170  |
| Butanol                                                           | cc. | 12.5 |

When all smell of solvents had disappeared, the paper of Example 2 was squeegeed on to the tacky surface, and the backing paper stripped away, leaving the emulsion adhering to the metal sheet. Adhesion was good during processing and when dry. During processing most of the triacetin was leached out, and the lacquer lost its tackiness, becoming hard.

It has been found that lacquered metal sheets to which emulsion layers have been transferred in accordance with this invention, have good keeping qualities. The emulsion does not tend to separate from the metal either during the photographic processing or when the layer is dried after processing. There is little or no tendency for the emulsion to "creep" on the metal, a phenomenon sometimes observed with other methods of making sensitised metal sheets.

A further and very important advantage of the use of transfer material in accordance with this invention is that the emulsions cut more smoothly than normal gelatin emulsions with less tendency to chip or tear around the line of the cut, a matter of considerable importance in the manufacture of templates.

While this invention primarily consists in the novel transfer material hereinbefore described, it also includes the method of sensitising sheets of metal, wood, plastic or other material hereinbefore described and the method of making templates and similar articles wherein a latent image in an emulsion transferred to a metal or other support as described, is processed, and the metal is cut to a form dictated by the resulting photographic image.

What I claim is:

1. A photographic transfer material adapted for lamination of the emulsion layer directly to the lacquered surface of a template comprising the following layers in order: a temporary support layer, an adhesive dry stripping layer and a layer of a photographic emulsion said latter layer being composed of light-sensitive silver halides dispersed in an ionic complex formed between gelatin and a compound selected from the group consisting of anion soaps and sulphonate acids containing a highly hydrophobic radical in the anion, said complex being the essential binding agent for the silver halide grains and being soluble in a solution composed of methyl alcohol.

2. A photographic transfer material adapted for lamination of the emulsion layer directly to the lacquered surface of a template comprising the following layers in order: a paper support layer, an adhesive dry stripping layer and a layer of a photographic emulsion said latter layer being composed of light-sensitive silver halides dispersed in an ionic complex formed between gelatin and a compound selected from the group consisting of anion soaps and sulphonate acids containing a highly hydrophobic radical in the anion, said complex being the essential binding agent for the silver halide grains and being soluble in a solution composed of methyl alcohol.

3. A photographic transfer material adapted

for lamination of the emulsion layer directly to the lacquered surface of a template comprising the following layers in order: a paper support layer, an adhesive dry stripping layer and a layer of a photographic emulsion said latter layer being composed of light-sensitive silver halides dispersed in an ionic complex formed between gelatin and a compound selected from the group consisting of anion soaps and sulphonic acids containing a highly hydrophobic radical in the anion, said complex being the essential binding agent for the silver halide grains and being soluble in a solution composed of methyl alcohol, and containing a proportion of an organic solvent-soluble colloid of a different type from said complex.

4. A photographic transfer material adapted for lamination of the emulsion layer directly to the lacquered surface of a template comprising the following layers in order: a paper support layer, an adhesive dry stripping layer and a layer of a photographic emulsion said latter layer being composed of light-sensitive silver halides dispersed in an ionic complex formed between gelatin and a compound selected from the group consisting of anion soaps and sulphonic acids containing a highly hydrophobic radical in the anion, said complex being the essential binding agent for the silver halide grains and being soluble in a solution composed of methyl alcohol, and containing a proportion of an organic solvent soluble cellulose derivative.

JOHN ALFRED HENRY HART.

### REFERENCES CITED

The following references are of record in the file of this patent:

#### UNITED STATES PATENTS

| Number       | Name            | Date          |
|--------------|-----------------|---------------|
| 2,118,059    | Slack et al.    | May 24, 1938  |
| 2,142,311    | Heidenhain      | Jan. 3, 1939  |
| 2,275,727    | Carroll et al.  | Mar. 10, 1942 |
| 10 2,282,001 | Russell et al.  | May 5, 1942   |
| 2,326,058    | Nadeau          | Aug. 3, 1943  |
| 2,362,593    | Staehle         | Nov. 14, 1944 |
| 2,386,602    | Gioseffi        | Oct. 9, 1945  |
| 15 2,409,564 | Heinecke et al. | Oct. 15, 1946 |
| 2,415,442    | Rackett         | Feb. 11, 1947 |
| 2,489,341    | Waller et al.   | Nov. 29, 1949 |

#### FOREIGN PATENTS

| Number     | Country       | Date          |
|------------|---------------|---------------|
| 29 537,256 | Great Britain | Oct. 12, 1940 |
| 554,300    | Great Britain | June 28, 1943 |
| 554,301    | Great Britain | June 28, 1943 |
| 556,360    | Great Britain | Oct. 1, 1943  |

#### OTHER REFERENCES

25 Journal of the American Chemical Society, December 1943, pages 2187-2190; May, 1944, pages 692-697.